

## UNITED STATES PATENT OFFICE

2,304,093

## REMOVING IRON FROM MAGNESIUM ALLOYS

Graydon E. Holdeman, Midland, Mich., assignor  
to The Dow Chemical Company, Midland,  
Mich., a corporation of Michigan

No Drawing. Application December 16, 1941,  
Serial No. 423,183

4 Claims. (Cl. 75—67)

This invention relates to the removal of iron impurities from magnesium-base alloys.

For some time it has been appreciated that the tendency of uncoated articles of magnesium-base alloys to corrode on exposure to moist air and to aqueous solutions is in some way dependent upon the presence of traces of iron in the metal. More recently, it has been shown that there is a certain minute but critical proportion of iron, e. g., about 0.002 per cent in the case of magnesium-base alloys containing aluminum, below which these metals are highly corrosion-resistant, but above which they are relatively corrodible. It is evident, then, that, in order to render iron-contaminated magnesium-base alloys resistant to attack, the iron content thereof must be reduced to below the critical corrosion tolerance limit. Unfortunately, however, since at least part of the iron is in actual physical solution in the metal when molten, many of the removal processes described in the art are ineffective in reducing the iron concentration to a sufficiently low value.

It is accordingly an object of the present invention to provide a simple and convenient method of treating iron-contaminated magnesium-base alloys to reduce the concentration of iron therein to a proportion well below the critical corrosion tolerance limit, i. e., to below about 0.002 per cent for most alloys.

The invention depends upon the discovery that iron is virtually insoluble, i. e., soluble to an extent well below 0.002 per cent by weight, in molten magnesium-base alloys containing a small proportion of beryllium. Thus, when beryllium is incorporated into the molten iron-contaminated alloy, the dissolved iron is rendered insoluble and precipitates, until less than 0.002 per cent remains in solution. The resulting alloy, since it contains iron in a proportion below the critical corrosion limit, is highly corrosion-resistant.

In removing dissolved iron impurities from iron-contaminated magnesium-base alloys according to the invention, then, the metal to be purified is first melted, ordinarily under a protective saline flux. Beryllium is then incorporated into the molten alloy in a proportion sufficient to precipitate the iron impurities, as by agitating the melt with metallic beryllium, usually in the form of a finely-divided beryllium-containing alloy, e. g., an aluminum-beryllium alloy. Alternatively, a small proportion of a reducible beryllium compound, conveniently anhydrous beryllium chloride, may be stirred into the molten

5 magnesium-base alloy, the compound being reduced to form metallic beryllium, which becomes incorporated into the melt. Following incorporation of the beryllium, whereby the iron impurities are rendered insoluble and precipitate, the molten alloy is separated from the precipitated iron impurities, usually by maintaining the melt quiescent for a time sufficient to allow the insoluble impurities to settle out of suspension, 10 and then decanting or ladling off the supernatant substantially iron-free alloy.

The initial proportion of beryllium to be incorporated into the molten magnesium-base alloy to effect precipitation of the iron impurities 15 varies slightly for different alloys, but is in general at least about 0.005 per cent by weight; a part of this beryllium may settle out of the melt during the iron-settling operation, even if no beryllium in excess of this value is originally present. With an initial beryllium concentration 20 in the metal of about 0.005 per cent, the iron impurities settle out of suspension usually within a few hours; higher initial concentrations of beryllium, approaching the maximum which 25 can be incorporated in the molten alloy, viz., 0.01 to 0.02 per cent, decrease the iron-settling time to a comparatively short period, often 0.2 to 1.0 hour. In general, the presence of sufficient beryllium is insured by agitating the melt with beryllium in a substantial excess of the requisite 30 0.005 per cent. Usually 0.1 to 0.2 per cent by weight of beryllium is added as beryllium chloride, or, in the treatment of aluminum-containing magnesium alloys, as an aluminum-beryllium alloy 35 containing 1 to 30 per cent of beryllium; with such excess, only a small part of the added beryllium actually becomes incorporated into the metal, probably by actual physical solution therein; the remainder of the beryllium is merely in suspension, and settles out the melt when agitation is discontinued.

The temperature of the molten alloy during the beryllium treatment is conveniently well above the melting point of the metal. In general, temperatures of about 1600° to 1700° F. permit more rapid iron-settling, although temperatures as low as 1350° F. or even less are operable. At the lower temperatures, the concentration of beryllium remaining in the metal after iron removal is lower than at the higher temperatures. If desired, the metal may be superheated at temperatures above 1600° F. to effect grain refinement without effecting the iron-settling.

The following examples will illustrate the invention:

*Example 1*

A magnesium-base alloy containing 5.4 per cent by weight of aluminum and 0.2 per cent of manganese, the balance being commercial magnesium, and containing at least 0.030 per cent iron impurity, was melted under a protective saline flux and heated to a temperature of 1500° F. Beryllium in a proportion of 0.04 per cent by weight of the alloy was then added with agitation in the form of an aluminum-beryllium alloy containing 10 per cent beryllium, the melt being heated to a temperature of 1700° F. to insure complete dispersion of the beryllium. The melt was then maintained quiescent and allowed to cool to a temperature of 1400° F. during a period of 50 minutes, during which time the iron impurities and most of the added beryllium settled out of suspension. The supernatant metal was ladled into iron-free molds and allowed to solidify. On analysis, the metal was found to contain 0.0009 per cent iron and 0.0031 per cent beryllium.

*Example 2*

A magnesium-base alloy containing 5.6 per cent by weight of aluminum and 3.0 per cent of zinc, the balance being commercial magnesium, and containing at least 0.030 per cent iron impurity, was melted under a protective flux and heated to a temperature of 1700° F. Beryllium in a proportion of 0.2 per cent by weight was added in the form of an aluminum-beryllium alloy containing 10 per cent of beryllium. The resulting melt was then stirred vigorously for 0.5 hour, after which it was held quiescent at 1700° F. for a few minutes to allow the iron impurities and most of the added beryllium to settle out of suspension. The resulting supernatant melt was then poured into molds and allowed to solidify. On analysis, the metal was found to contain 0.0002 per cent iron and somewhat over 0.01 per cent beryllium.

It should be explained that the precise analytical determination of minute proportions of beryllium in magnesium alloys is difficult, and that the numerical values of beryllium concentration set forth above are therefore only the best approximations available. All beryllium concentrations herein reported were determined by painstaking application of standard spectrochemical procedures.

The foregoing description is illustrative rather

than strictly limitative, the invention being co-extensive in scope with the following claims.

I claim:

1. The method of removing dissolved iron impurities from molten iron-contaminated magnesium-base alloys which comprises incorporating beryllium into the molten metal in a proportion sufficient to precipitate the iron impurities, and separating the precipitated impurities from the molten metal.

2. The method of removing dissolved iron impurities from molten iron-contaminated magnesium-base alloys which comprises agitating the molten metal with a sufficient quantity of a substance selected from the class consisting of beryllium and reducible beryllium compounds to incorporate therein at least about 0.005 per cent by weight of beryllium, whereby the iron impurities are rendered insoluble and precipitate; and separating the molten metal from the precipitated iron impurities.

3. The method of removing dissolved iron impurities from molten iron-contaminated magnesium-base alloys which comprises agitating the molten metal with a sufficient quantity of a substance selected from the class consisting of beryllium and reducible beryllium compounds to incorporate therein at least about 0.005 per cent by weight of beryllium, whereby the iron impurities are rendered insoluble and precipitate; discontinuing agitation and maintaining the melt quiescent for a time sufficient to permit the insoluble iron impurities to settle out of suspension; and separating the supernatant iron free metal from the settled impurities.

4. The method of treating an iron-contaminated aluminum-containing magnesium-base alloy to remove the iron therefrom to a value below 0.002 per cent which comprises agitating the molten metal with a small proportion of an aluminum-beryllium alloy in a quantity sufficient to incorporate into the melt at least about 0.005 per cent beryllium, whereby the iron impurities are rendered insoluble and precipitate; discontinuing agitation and maintaining the melt quiescent for a time sufficient to permit the insoluble iron impurities to settle out of suspension; and separating the supernatant iron-free metal from the settled impurities.

GRAYDON E. HOLDEMAN.